

Feb. 12, 1957

M. C. M. GRANDPIERRE  
PROCESS AND APPARATUS FOR THE TREATMENT  
OF MOLTEN FERROUS ALLOYS

Filed March 3, 1955

2,781,260

6 Sheets-Sheet 1



INVENTOR.

MAURICE C. M. GRANDPIERRE

BY

*C. Dr. Deller*  
ATTORNEY

Feb. 12, 1957

Feb. 12, 1957 M. C. M. GRANDPIERRE  
PROCESS AND APPARATUS FOR THE TREATMENT  
OF MOLTEN FERROUS ALLOYS  
Filed March 3, 1955 69

2,781,260

6 Sheets-Sheet 2

Fig. 2.



Fig. 3.



INVENTOR.  
*MAURICE C. M. GRANDPIERRE*

BY

*C. Ar. Deller*  
ATTORNEY

Feb. 12, 1957

Feb. 12, 1957 M. C. M. GRANDPIERRE  
PROCESS AND APPARATUS FOR THE TREATMENT  
OF MOLTEN FERROUS ALLOYS  
Filed March 3, 1955 6

2,781,260

Filed March 3, 1955

6 Sheets-Sheet 3



INVENTOR.  
*MAURICE C.M. GRANDPIERRE*  
R.V.

BY  
C. Ar. Deller  
ATTORNEY

Feb. 12, 1957

M. C. M. GRANDPIERRE  
PROCESS AND APPARATUS FOR THE TREATMENT  
OF MOLTEN FERROUS ALLOYS

2,781,260

Filed March 3, 1955

6 Sheets-Sheet 4



*Fig. 8.*



*Fig. 9.*



INVENTOR.

MAURICE C. M. GRANDPIERRE  
BY

*C. Dr. Deller*  
ATTORNEY

Feb. 12, 1957

M. C. M. GRANDPIERRE  
PROCESS AND APPARATUS FOR THE TREATMENT  
OF MOLTEN FERROUS ALLOYS

2,781,260

Filed March 3, 1955

6 Sheets-Sheet 5



Feb. 12, 1957

M. C. M. GRANDPIERRE  
PROCESS AND APPARATUS FOR THE TREATMENT  
OF MOLTEN FERROUS ALLOYS

Filed March 3, 1955

2,781,260

6 Sheets-Sheet 6



INVENTOR.  
MAURICE C.M. GRANDPIERRE

BY

C. R. Decker  
ATTORNEY

# United States Patent Office

2,781,260

Patented Feb. 12, 1957

1

2,781,260

## PROCESS AND APPARATUS FOR THE TREATMENT OF MOLTEN FERROUS ALLOYS

Maurice Charles Marie Grandpierre, Pont-a-Mousson, Nancy, France, assignor to The International Nickel Company, Inc., New York, N. Y., a corporation of Delaware

Application March 3, 1955, Serial No. 491,820

Claims priority, application France March 6, 1954

18 Claims. (Cl. 75—130)

The present invention is directed to the treatment of a liquid ferrous alloy such as cast iron and steel and, more particularly, to an improved method for introducing into such a liquid ferrous alloy an addition element having desulfurizing properties.

It has been heretofore proposed to introduce addition elements having desulfurizing properties into liquid ferrous alloys to improve the quality of the resulting castings. It has also been discovered that many reactive elements having desulfurizing properties when used in the treatment of molten cast iron have the ability to control graphite occurring in the resulting castings to a spheroidal form with accompanying great improvement in the mechanical properties of the castings. It has been known that addition elements having desulfurizing properties, e. g., magnesium, cerium, calcium, etc., are quite oxidizable and have low boiling points compared with the temperature of the liquid ferrous alloy. The result of this is that, in spite of the precautions that it has already been found possible to take by following various known procedures for introducing these elements, such as operating in an atmosphere which does not react with the addition element or by plunging the addition element into the interior of the ferrous alloy either with or without the presence of a neutral atmosphere, the losses by volatilization and/or combustion of the addition element are considerable. The final result of this is that with a given total quantity of the element introduced, there remains in each case and by all known procedures a high degree of uncertainty regarding the final content of the addition element in the alloy.

To such an extent is this true that, in practice, there are observable in the alloys obtained considerable differences—as between one heat and another—in behavior and properties. This involves the necessity of a permanent check on every heat and a need to provide considerable margins of safety.

It has now been discovered that when a reactive element is introduced into a molten ferrous alloy under highly specialized conditions, the addition reactions are placed under rigid control with resulting high recovery of the reactive addition agents in the molten ferrous alloy.

It is an object of the invention to provide an improved method for introducing reactive elements into molten ferrous alloys.

It is a further object of the invention to provide a method for introducing desulfurizing agents into molten cast iron in a particularly effective manner.

Another object of the invention is to provide a special apparatus adapted for the purpose of introducing reactive agents having desulfurizing properties into molten ferrous alloys.

Other objects and advantages of the invention will become apparent from the following description taken in conjunction with the accompanying drawings in which:

Figure 1 depicts the design of an apparatus constructed in accordance with the present invention and adapted for the purpose of introducing reactive desulfurizing agents into molten ferrous metals;

2

Fig. 2 is a horizontal view of a portion of the apparatus depicted in Figure 1 with the apparatus being shown in the open position;

Figure 3 is a view on an enlarged scale of an immersion container utilized for introducing the reactive addition alloy;

Figure 4 is a partial view in elevation of a first variant with a device for stirring by induction;

Figure 5 is a similar view of a second variant;

Figure 6 is a view in perspective of an immersion container of this second variant;

Figure 7 is a partial view in elevation of a third variant;

Figures 8 and 9 are horizontal sections along lines VIII—VIII and IX—IX of Figure 7 but on a larger scale;

Figure 10 is an elevation, partly in section, of a further apparatus;

Figure 11 is a section on the line XI—XI in Figure 10;

Figure 12 is a section on the line XII—XII in Figure 10; and

Figure 13 is an elevation of apparatus, essentially as shown in Figure 10, mounted on a carriage.

Broadly stated, the present invention is directed to a method for introducing reactive addition metals having desulfurizing properties into molten ferrous metal while the molten ferrous metal is subjected to substantial pressure and while the molten ferrous metal is being stirred. The pressure utilized in accordance with the invention preferably is generated by introducing into the space above the molten ferrous metal a gas under high pressure.

30 In the invention, the introduction of the addition element is effected in a closed vessel maintained under a gas pressure at least equal to the vapor pressure of the addition element at the temperature within the vessel so that the addition element is liquefied, and the molten metal is vigorously stirred to mix the liquid addition element with the molten metal. The liquefied addition agent will normally float on the molten iron or steel, and the stirring ensures that intimate mixing takes place despite the tendency to float. If more than one addition element is

35 to be introduced, the pressure in the vessel is maintained above that of the addition element with the highest vapor pressure. It is found possible in this way to retain in the solidified metal a greater proportion of a highly volatile addition agent than has been possible hitherto, and also to control more effectively than hitherto the actual amount of the addition agent retained in the solidified metal.

40 The result of this is that it is possible, for a given desired content, to know in advance with an adequate degree of accuracy the total amount of the addition element to be introduced, account being taken of unavoidable small losses, such as those due to partial evaporation of some of the addition element during the course of the treatment and those due to slight condensations on the walls of the receptacle in which the treatment is effected.

45 The pressure in the vessel should be very high if the best results are to be obtained. For instance, molten iron to be cast is commonly at a temperature of the order of 1500° C. and at this temperature the vapor pressure of magnesium is about 185 lbs./in.<sup>2</sup>. In adding magnesium to molten iron at this temperature, therefore, it is necessary for the pressure to be higher than 185 lbs./in.<sup>2</sup> and preferably it is greater than 225 lbs./in.<sup>2</sup>.

50 To determine the pressure to be used for a particular addition element at the desired operating temperature, the Clapeyron equation, as given, for example, in "Basic Open Hearth Steelmaking," 1951 edition, page 537, may be employed. For magnesium this equation is:

$$\log P_{\text{atm}} = -\frac{32520}{4.575T} + 5.158$$

55 70 T being the absolute temperature in °C.

Pressures of this magnitude can easily be set up by introducing a compressed gas into the vessel. The gas used depends on the nature of the addition agent. If oxidation of the addition element must be prevented in order to prevent loss, the compressed gas should be inert, being preferably argon or nitrogen, and is recovered from the vessel after the mixing is complete for the sake of economy. On adding magnesium to molten iron according to the invention, however, it has surprisingly been found that if compressed air is used the loss of magnesium by oxidation is comparatively small and is more than balanced by the cheapness of compressed air and the simplification of the necessary apparatus.

A vessel equipped with a stirring device and constructed to withstand the high pressure involved cannot readily be used as a ladle into which the metal is poured. The process is therefore preferably carried out in an apparatus comprising a pressure vessel made in upper and lower parts, the upper part being movable to allow a ladle containing molten metal to be put in the lower part and thereafter to make a gas-tight closure with the lower part.

Generally speaking, the apparatus contemplated in accordance with the present invention comprises such a pressure vessel or jacket adapted to hold a ladle of the molten ferrous alloy to be treated, said vessel being provided with a gas-tight opening through which the molten metal to be treated and the addition material can be introduced, means for applying gaseous pressure upon the molten metal in said vessel and means for stirring the molten metal while said pressure is being applied thereto.

In order to give those skilled in the art a better understanding of the operation of the invention as adapted to the apparatus depicted in Figures 1 to 3, the following description is given:

The apparatus includes a pressure vessel 3 consisting of a lower part or body 6 and an upper part or a lid 11, the body being carried on a support 5 in a pit 2 which also contains a steel framework 1. The body 6 can be raised and lowered by an hydraulic ram 4. The lid 11 is carried by a frame 12 which can swing in a horizontal plane about a pin 13 in the top of the framework 1, which is made with a slot 14 engaging with a T-shaped projection 15 on the framework. In the position shown in Figure 1 the projection 15 lies in the slot 14, and the frame 12 therefore holds the lid 11 fixed. The ram forces the body 6 hard against the lid 11 to make a pressure-tight joint. In the position shown in Figure 2 the ram 4 has been lowered and the frame 12 swung horizontally to give free access to the interior of the body 6 of the vessel.

Operating fluid is supplied to and released from the ram 4 through a pipe 7 controlled by a three-way cock 8.

When the vessel 3 is open, a ladle 48 containing molten metal 49 can be put into or removed from the body 6. The bottom of the body 6 is recessed at 50 to receive and locate the ladle 48.

The lid 11 carries an openwork container 20 for the addition agent, and this also serves as a stirring device. The container 20 is a bell of graphite or of iron with a refractory coating and has openings 21 in its wall. Before the ladle is introduced into the vessel 3, addition agent 53, e. g. magnesium in small pieces, is put on an asbestos plate 52, and this plate is inserted through the open underside of the container and supported by a grid 22 which is held in position by rods 9. When the ladle is in the vessel 3, the container 20 is immersed in the molten metal, which then enters the container through the openings 21 and causes the addition agent to melt and flow out through the openings.

To allow the container 20 to be immersed in the molten metal, it is carried by a rod 19 mounted to slide through the upper part of the vessel and connected externally to a reciprocating piston 10. The rod 19 is secured by a collar 42 to a rod 18 which passes through the lid 11 and carries the piston 10 in a cylinder 17. This cylinder is fixed in a bridge 16 rigid with the frame 12 and so swings

with the frame. It is connected by flexible pipes 23 to a valve 24 which controls the supply of compressed air from a pipe 25 to the cylinder 17, each end of the cylinder being put under pressure in turn while the other end is exhausted to the atmosphere through a pipe 26. The valve 24 is operated by a solenoid 27 under control of a switch 28, opening and closing of the switch causing the valve, and therefore the piston 10 and the container 20, to reciprocate vertically.

10 The apparatus shown in Figure 1 is designed for operation with a non-oxidizing gas, e. g. argon. This is supplied from a high-pressure container 32 through a pipe 30 controlled by a valve 31 to an opening 29 in the body 6. In order to fill the vessel 3 with argon under high pressure, it is necessary first to expel the air, and this is done through an opening 39 in the lid 11, the opening being connected by a flexible pipe 40 to a three-way cock 41 which puts the pipe 40 into communication with the atmosphere during the air expulsion and subsequently is closed.

It will now be appreciated that the sequence of operations is to charge the container 20; insert the ladle 48 containing the molten metal 49 in the vessel 3; close the vessel by swinging the frame 12 and then operate the ram 4; expel the air by opening the valve 31 and turn the cock 41 to exhaust the air to atmosphere; close the cock 41 to allow the pressure in the vessel 3 to build up to the desired high value; close the switch 28 to lower the container 20 into the molten metal; and then repeatedly open 25 and close the switch 28 to cause the container 20 to reciprocate and stir the molten metal so as to mix the addition agent with it.

When the liquid metal makes contact with the addition element or elements, the latter melts with a tendency to evaporation. As, however, the pressure in the container is greater than the vapor pressure of this element at the temperature under consideration, it remains liquid. Owing to its low density, compared with that of the alloy being treated, the liquid element tends to float and it is 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665

In each test and example 200 kilograms of cast iron were treated, the addition agent being pure magnesium added in the proportion of 0.10%, i. e. 200 grams.

*Test I*

The molten iron contained:

| C       | Si      | Mn      | P       | S       |
|---------|---------|---------|---------|---------|
| Percent | Percent | Percent | Percent | Percent |
| 3.75    | 1.70    | 0.08    | 0.04    | 0.032   |

The temperature of the iron when introduced into the ladle 48 was 1440° C. as read from an optical pyrometer without compensation for emissivity (i. e. a true temperature of about 1500° C.). The mixing operation lasted 2 minutes, the argon pressure being maintained between 42 and 75 lbs./in.<sup>2</sup>. During this time the container 20 plunged up and down fifteen times. The temperature of the iron at the end of the operation was 1315° C. (as read). Analysis of the iron showed that the amount of magnesium retained was 0.01%, and the sulfur content was 0.017%. Microscopic examination revealed a flake graphite structure and mechanical properties equivalent to those of an ordinary gray cast iron. The magnesium recovery was 21%.

*Test II*

The molten iron contained:

| C       | Si      | Mn      | P       | S       |
|---------|---------|---------|---------|---------|
| Percent | Percent | Percent | Percent | Percent |
| 3.80    | 1.75    | 0.07    | 0.04    | 0.026   |

The temperature (as read) of the iron at the start of the operation was 1420° C. Mixing lasted 1½ minutes, the argon pressure being held between 130 and 145 lbs./in.<sup>2</sup>, i. e., still well below the vapor pressure of magnesium at the temperature of the iron. The retained magnesium content was 0.01% and the final sulfur content 0.008%. The magnesium recovery was thus 23%, and the graphite was in flake form.

*Test III*

The molten iron contained:

| C       | Si      | Mn      | P       | S       |
|---------|---------|---------|---------|---------|
| Percent | Percent | Percent | Percent | Percent |
| 3.73    | 1.72    | 0.07    | 0.04    | 0.03    |

The temperature (as read) of the iron at the start of the operation was 1450° C. The operation lasted 1½ minutes, the argon pressure being held between 155 and 178 lbs./in.<sup>2</sup>, i. e., slightly below the vapor pressure of magnesium. The final temperature (as read) was 1280° C. The retained magnesium content was 0.03% and the sulfur content 0.010%. The magnesium recovery was 45%. Microscopic examination still showed flake graphite, though some spheroids had formed.

*Example IV*

The molten iron contained:

| C       | Si      | Mn      | P       | S       |
|---------|---------|---------|---------|---------|
| Percent | Percent | Percent | Percent | Percent |
| 3.74    | 1.70    | 0.08    | 0.04    | 0.036   |

The temperature (as read) of the iron at the start of the operation was 1465° C. The operation lasted 2 minutes with an argon pressure between 225 and 268 lbs./in.<sup>2</sup>,

i. e., a pressure greater than the vapor pressure of magnesium. The final temperature (as read) was 1300° C. This iron was inoculated with 1% of ferro-silicon (75% Si) which gave a final silicon content of 2.43%. The retained magnesium content of the cast iron was 0.04% and the final sulfur content 0.007%. The magnesium recovery was thus 62% and the graphite was spheroidal.

10 A test piece 25 mm. thick, cast in dry sand from the inoculated iron, had a tensile strength, as cast, of 76 kg./mm.<sup>2</sup> (48 tons/in.<sup>2</sup>), an elongation at fracture of 4% and a Brinell hardness of 229.

*Example V*

The molten iron contained:

| C       | Si      | Mn      | P       | S       |
|---------|---------|---------|---------|---------|
| Percent | Percent | Percent | Percent | Percent |
| 3.75    | 1.80    | 0.07    | 0.04    | 0.031   |

15 The temperature (as read) of the iron at the start of the operation was 1470° C. The operation lasted 2 minutes in a nitrogen atmosphere, the pressure of which was between 225 and 254 lbs./in.<sup>2</sup>. The retained magnesium content was 0.05% and the sulfur content 0.007%. The recovery was thus 68%, and microscopic examination showed spheroidal graphite. The mechanical properties of the iron, as cast, were approximately equivalent to those of the iron obtained in Example IV.

20 25 The above-cited Examples IV and V show that application of this procedure in accordance with the invention enables contents of magnesium to be obtained which ensure the presence of graphite in spheroidal form in cast iron as a result of quite small additions (0.10%) of magnesium to molten cast iron. Furthermore, the use of magnesium in the pure state ensures economical manufacture. The tests and examples also show clearly that the results desired are only obtained with a treating pressure which is at least equal to the vapor pressure of the addition element at the temperature of the treatment. Those skilled in the art will appreciate that the maximum pressure employed is a practical consideration influenced by the strength of the materials used in the apparatus and the requirements of the particular application.

25 30 35 40 45 50 55 60 Stirring of the cast iron or other ferrous alloy during treatment can, of course, be effected by other means than that described in the course of Test I. There is shown in Figure 4 a first variant in which stirring is obtained by electrical induction, a device already known as such. For this to be done, the vessel 3 is provided inside with a winding 54 suitably insulated from the wall of the container and connected with a high frequency generator 55. The rest of the apparatus is identical with that in Figure 1. It may be noted that, in view of the stirring obtained by means of the winding 54, it is not necessary during the treatment to move the bell containing the addition element or elements.

65 70 75 Figures 5 and 6 illustrate another variant in which the container 20 is carried by a shaft 34 mounted to slide through the upper part of the vessel and externally connected to a motor 56, so that the container can be rotated within the metal 49. To ensure adequate stirring the container 20 is provided with vanes 57. The motor 56 and shaft 34 can be moved up and down as a unit by a piston 10 on a shaft 18 secured to a frame 36 in which the motor is mounted. In this variant the rest of the apparatus is identical with that in Figure 1.

75 80 85 90 Figures 7 to 9 illustrate another variant in which the vessel 3 has dimensions enabling it to receive two ladles, one on top of the other. The molten metal is allowed to run out of the upper ladle 62 onto pieces of magnesium 53 in the lower ladle 58. These pieces are held down by a perforated plate 60 with peripheral notches 61 shaped

to pass axially past lugs 59, the plate, after partial rotation, being held by the lugs against axial movement.

The molten metal in the upper ladle 62 can pass through a hole in the bottom of the ladle when a plug 63 is removed. This plug is in position when the ladle is put in the vessel 3 and its upper end is pivoted to a lever 64. This lever is pivoted on the ladle 62, and after the ladle has been put in the vessel 3 the free end of the lever 64 is in contact with a disc 65 on a rod 19 similar to the rod 19 in Figure 1. Then downward movement of the disc 65 rocks the lever and lifts the plug 63. The metal flows into the ladle 58 and the magnesium retained by the plate 60 melts progressively, flowing through the metal, which is stirred by the further metal entering from the ladle 62.

When compressed air can be used to set up the pressure, it is possible to use the much simpler apparatus shown in Figures 10 to 13. This also includes yet another form of stirring device.

In this apparatus a pressure vessel 109 consists of a relatively shallow lower part 101 and a relatively large upper part 109. The lower part 101 has a refractory lining 102 and lugs 103 which locate and support a ladle 48 containing molten metal 49. The upper edge of the part 101 is frusto-conical as shown at 107 to mate with a complementary surface on the upper part 109, which carries a heat-resistant packing 113 to ensure a tight joint between the two mating surfaces. The part 109 has a flange 110 and the lower part 101 has lugs 108. A ring 114, U-shaped in cross-section, surrounds the flange 110 and the lower arm of the U is recessed to clear the lugs 108 on axial movement. On turning the ring 114 the lower arm of the U engages beneath the lugs 108 to hold the parts 101 and 109 together. The engaging surfaces of the ring 114 and lugs 108 are slightly inclined to produce a wedging action when the ring 114 is turned.

The ring 114 is turned mechanically by a pneumatic ram 115 having a casing connected by a lever 116 to the part 109 and a plunger 117 connected to the ring at 118. The stroke of the ram plunger is such as to bring the ring either into the position in which the lugs 108 can pass through the recesses in the ring or into the position in which the parts 101 and 109 of the vessel are urged towards one another to the maximum extent.

The upper part 109 of the vessel in this apparatus has a throat 120 leading to a compartment 119 closed by a cover plate 121 and housing a rod 122 carrying a stirring device 126. This device is a disc and differs essentially from the device 29 of Figure 1 in that it does not contain the addition agent. The addition agent 150, in stick form, is introduced into the part 109 through an opening 141 above the disc 126 while the disc is in its uppermost position shown in dotted lines. The disc supports the addition agent 150 and keeps it from falling into the molten metal 49 until the disc is moved downwards. The opening 141 is closed by a cover plate 142.

The stirring device 126, the rod 122 of which has a refractory covering 127 and carries a centering collar 125, is articulated to a double-armed lever 123 which is rigid with a pivot mounting 124 which passes in fluid-tight fashion through the upper part 109 of the vessel. The lever 123 carries a counterweight 129 and is rocked by an hydraulic ram 131 pivotally mounted on the outside of the upper part 109 of the vessel with its plunger pivotally connected to the lever 123. It will be seen that by causing the ram to reciprocate, the stirring device 126 is first moved downward to allow the addition agent 150 to fall into the ladle 48 and then is moved up and down with some rocking movement in the molten metal, to stir it. To ensure that a magnesium addition agent will readily dissolve in molten iron, the speed of movement of the disc 126 should be about 6 inches per second.

A compressed air reservoir 134 is mounted on a bracket 133 on the part 109 and is fed through a pipe 135 controlled by a valve 136. This reservoir is connected to the interior of the vessel 100 by a passage 137 of substantial

cross-section, controlled by a valve 138. The size of this passage allows the vessel to be put under pressure quickly. At the end of the mixing the pressure can be released by opening a valve 140 in an outlet 139 also of substantial cross-section.

The upper part 109 of the vessel can be lifted by a hook 145 on the end of a cable 143 which carries a counterweight 144 and runs over a pulley 146 and a drum 147 on a rotary beam 148. The drum 147 can be turned by an electric motor 128. The beam 148 which supports the cable can turn on a pillar 149. The upper part 109 can therefore be lowered in succession onto different lower parts 101 arranged around the pillar 149, each lower part containing a ladle of molten metal to be treated. Figure 13 shows two lower vessel parts 101A and 101B mounted on a carriage 151 which can run between end positions determined by chocks 152 and 153 to bring each lower part in turn beneath an upper part 109 arranged to be lifted and lowered by a lifted mechanism fixed in position.

The apparatus shown in Figures 10 to 13 presents the advantage that the time taken by the operations preliminary to the treatment proper with the addition agent is very considerably reduced and thus the metal is at a higher temperature for casting when the mixing is complete. Moreover, with energetic stirring by the device 126 the time of mixing is also reduced, say to 1 minute or 1½ minutes, thus reducing the loss of addition agent by oxidation and by condensation on the walls of the pressure vessel.

The results of two processes carried out according to the invention with the apparatus shown in Figure 10 will now be given. As in the earlier tests and examples, 200 grams of magnesium were added to 200 kgs. of molten iron in each case.

#### Example VI

The molten iron contained:

| C               | Si              | Mn              | P               | S                |
|-----------------|-----------------|-----------------|-----------------|------------------|
| Percent<br>3.85 | Percent<br>1.72 | Percent<br>0.05 | Percent<br>0.05 | Percent<br>0.016 |

The temperature of the molten metal (as read) was 1420° C. at the time of closing of the vessel 100. The total duration of the operation was 3 minutes, and that of the actual mixing 75 seconds, the air pressure being between 225 and 254 lbs./in.<sup>2</sup>. At the end of the operation the temperature (as read) was 1350° C., i. e. a drop of only 70° C.

The iron as cast contained 0.044% retained magnesium and 0.008% sulfur, so the magnesium recovery was 50%. The graphite was all spheroidal.

#### Example VII

The molten iron contained:

| C              | Si             | Mn              | P               | S                |
|----------------|----------------|-----------------|-----------------|------------------|
| Percent<br>3.6 | Percent<br>1.7 | Percent<br>0.07 | Percent<br>0.04 | Percent<br>0.019 |

The temperature (as read) when the vessel was closed was 1430° C. The total duration of the operation was 2½ minutes, the mixing occupying one minute, and the air pressure was between 239 and 268 lbs./in.<sup>2</sup>. The final temperature (as read) was 1370° C., the fall in temperature being thus only 60° C. The retained magnesium content was 0.049% and the final sulfur content 0.008%, so the magnesium recovery was 57%. All the graphite was spheroidal.

The apparatus may be modified further in that the lower part may be no more than a plate-like support for a ladle, and the upper part may be a bell wholly surrounding the ladle.

Naturally if the apparatus shown in Figures 10 to 13 is to be used with a non-oxidising gas, a gas-recovery system similar to that shown in Figure 1 may be added.

The method and apparatus contemplated in accordance with the invention may be used for the purpose of desulfurizing ferrous alloys or may be used for the purpose of producing alloys of ferrous metals, such as cast iron and steel containing one or more metals, having desulfurizing properties in ferrous metal. As has previously been mentioned herein, magnesium, calcium and cerium are elements having such desulfurizing properties. Those skilled in the art will appreciate that other members of the alkali and alkaline earth metal groups, etc., also are recognized to have such desulfurizing properties. These metals all have melting points lower than that of iron. It will be appreciated that when desulfurization is the primary object then quite small amounts of the reactive elements may be employed. Thus, in the case of magnesium, an amount of magnesium approximately equal on a weight basis to the amount of sulfur in the metal, e. g., cast iron being treated, is usually sufficient to effect desulfurization. When it is desired to produce alloys containing the reactive metal then somewhat larger additions of reactive metal are employed. For example, in the case of magnesium, amounts of magnesium on the order of up to about 0.5% may be added to the molten cast iron in accordance with the present invention.

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

I claim:

1. The method for introducing a reactive metal into a molten ferrous alloy which comprises applying to a bath of said molten alloy a gas pressure at least equal to the vapor pressure of the reactive metal at the temperature of said molten alloy, inserting a reactive metal beneath the surface of said molten alloy and energetically stirring said molten alloy in contact with said reactive metal until substantially all of said reactive metal has become incorporated in said molten alloy.

2. The method for alloying molten metal from the group consisting of cast iron and steel with a reactive metal from the group consisting of magnesium, calcium and cerium which comprises establishing a bath of metal from the group consisting of cast iron and steel, applying to said bath a gas pressure at least equal to the vapor pressure at the temperature of said bath of the reactive metal added, inserting a reactive metal from the group consisting of magnesium, calcium and cerium into said bath and energetically stirring said bath while maintaining said pressure for sufficient time to incorporate said reactive metal substantially in said bath.

3. The process for introducing magnesium into molten cast iron which comprises establishing a bath of molten cast iron, applying thereto a gas pressure at least equal to about the vapor pressure of magnesium at the temperature of said molten cast iron, inserting magnesium into said molten bath and agitating said bath while applying gas pressure thereto until the alloying of magnesium with the molten cast iron is effected.

4. The process for introducing magnesium into molten cast iron which comprises establishing a bath of molten cast iron, applying thereto an air pressure at least equal to about the vapor pressure of magnesium at the temperature of said molten cast iron, inserting magnesium into said molten bath and agitating said bath while applying

said air pressure thereto until the alloying of magnesium with the molten cast iron is effected.

5. The process for introducing magnesium into molten cast iron which comprises establishing a bath of molten cast iron, applying thereto a substantially non-oxidizing gas at a pressure at least equal to about the vapor pressure of magnesium at the temperature of said molten cast iron, inserting magnesium into said molten bath and agitating said bath while applying said gas pressure thereto until the alloying of magnesium with the molten cast iron is effected.

10 6. The process for introducing magnesium into molten cast iron which comprises establishing a bath of molten cast iron, applying thereto argon gas at a pressure at least equal to about the vapor pressure of magnesium at the temperature of said molten cast iron, inserting magnesium into said molten bath and agitating said bath while applying pressure thereto until the alloying of magnesium with the molten cast iron is effected.

20 7. The process for introducing magnesium into molten cast iron which comprises establishing a bath of molten cast iron, applying thereto air at a pressure of at least about 225 lbs. per square inch, inserting magnesium into said molten cast iron and agitating said molten cast iron while maintaining said pressure until said magnesium is alloyed with said molten cast iron.

30 8. An apparatus adapted for the treatment of molten metal under pressure of a gas whereby said gas may be recovered which comprises, in combination, a pressure vessel adapted to hold molten metal, a source of high-pressure gas connected to said pressure vessel by a control valve, a low-pressure reservoir connected to said pressure vessel by a control valve and a compressor connected between said low-pressure reservoir and said high-pressure source, said compressor being adapted to pump gas from said low-pressure reservoir to said high-pressure source and thereby to recover gas received in said low-pressure reservoir.

35 9. An apparatus particularly adapted for the introduction of reactive metals into molten ferrous melts and comprising, in combination, a pressure vessel having an opening provided with a gas-tight closure, a container for holding molten metal disposed within said vessel, means for introducing gas under high pressure into said vessel, means for controllably introducing addition material below the surface of molten metal held in said vessel, and a high-frequency induction coil disposed about the molten metal container whereby stirring is effected by electromagnetic induction.

40 10. An apparatus adapted for the treatment of molten metal comprising, in combination, a vessel having a lid and being adapted to hold molten metal under pressure, means for supplying gas pressure within said vessel, and a receptacle disposed within said vessel and adapted to hold addition material, said receptacle being provided with outer vanes and being connected through said lid with means for imparting rotational motion to said receptacle.

45 11. An apparatus adapted for the treatment of molten metal under pressure which comprises, in combination, a pressure vessel adapted to hold molten metal, a source of high-pressure gas connected to said vessel, and mixing means disposed within the pressure vessel and having two ladles placed one atop the other, with the lower ladle adapted initially to contain addition material, and with the upper ladle being provided with a stopper openable from without the vessel.

50 12. An apparatus adapted for the introduction of reactive metals into molten ferrous alloys and comprising a pressure vessel made in upper and lower parts, the upper part being removable to allow a ladle containing molten metal to be placed in a lower part and thereafter to make a gas-tight closure with said lower part, means for placing the interior of the closed vessel under gas pressure, means for introducing an addition element into the metal

## 11

in the ladle after the closing of the vessel, and means for bringing about vigorous stirring of the metal in the ladle while the vessel is closed, the stirring means being a disc mounted in its uppermost position to support an addition agent introduced through an opening above it, whereby on downward movement of the disc the addition agent is allowed to enter the metal and the metal is stirred by the disc.

13. An apparatus adapted for the introduction of reactive metals into molten ferrous alloys and comprising a pressure vessel made in upper and lower parts, the upper part being removable to allow a ladle containing molten metal to be placed in a lower part and thereafter to make a gas-tight closure with said lower part, means for placing the interior of the closed vessel under gas pressure, means for introducing an addition element into the metal in the ladle after the closing of the vessel, and means for bringing about vigorous stirring of the metal in the ladle while the vessel is closed, the stirring means being articulated to a double-armed lever having a pivot mounting which passes through the upper part of the vessel, the lever being rocked by a device itself mounted on the outside of the upper part of the vessel.

14. An apparatus adapted for the introduction of reactive metals into molten ferrous alloys and comprising a pressure vessel made in upper and lower parts, the upper part being removable to allow a ladle containing molten metal to be placed in a lower part and thereafter to make a gas-tight closure with said lower part, means for placing the interior of the closed vessel under gas pressure, means for introducing an addition element into the metal in the ladle after the closing of the vessel, and means for bringing about vigorous stirring of the metal in the ladle while the vessel is closed, the upper part of the vessel being engageable by a hook on a lifting cable carried by a rotary support, whereby the upper part can be lowered onto different lower parts in succession.

15. An apparatus adapted for the introduction of reactive metals into molten ferrous alloys and comprising a pressure vessel made in upper and lower parts, the upper part being removable to allow a ladle containing molten metal to be placed in a lower part and thereafter to make a gas-tight closure with said lower part, means for placing the interior of the closed vessel under gas pressure, means for introducing an addition element into the metal in the ladle after the closing of the vessel, and means for bringing about vigorous stirring of the metal in the ladle

## 12

while the vessel is closed, two or more lower vessel parts being mounted on a carriage which carries them in turn beneath a single upper part.

16. An apparatus adapted for the introduction of reactive metals into molten ferrous alloys and comprising a pressure vessel made in upper and lower parts, the upper part being removable to allow a ladle containing molten metal to be placed in a lower part and thereafter to make a gas-tight closure with said lower part, means for placing the interior of the closed vessel under gas pressure, means for introducing an addition element into the metal in the ladle after the closing of the vessel, and means for bringing about vigorous stirring of the metal in the ladle while the vessel is closed, the upper and lower parts of the vessel presenting conical mating surfaces, one of which is recessed to receive a packing.

17. An apparatus adapted for the introduction of reactive metals into molten ferrous alloys and comprising a pressure vessel made in upper and lower parts, the upper part being removable to allow a ladle containing molten metal to be placed in a lower part and thereafter to make a gas-tight closure with said lower part, means for placing the interior of the closed vessel under gas pressure, means for introducing an addition element into the metal in the ladle after the closing of the vessel, and means for bringing about vigorous stirring of the metal in the ladle while the vessel is closed, the two parts of the vessel interengaging by relative axial movement followed by rotary movement of a locking ring on one part into engagement with fixed lugs on the other part, and a power-actuated device being provided on the first part to turn the locking ring.

18. The process for introducing magnesium into molten cast iron which comprises establishing a bath of molten cast iron, applying thereto air at a pressure of at least about 185 pounds per square inch, inserting magnesium into said molten cast iron and agitating said molten cast iron while maintaining said pressure until said magnesium is alloyed with said molten cast iron.

## References Cited in the file of this patent

## UNITED STATES PATENTS

|            |               |               |
|------------|---------------|---------------|
| Re. 13,849 | Simpson       | Dec. 15, 1914 |
| 1,707,161  | Hoy           | Mar. 26, 1929 |
| 1,808,145  | Machlet       | June 2, 1931  |
| 2,485,760  | Millis et al. | Oct. 25, 1949 |